# EUROPEAN PATENT SPECIFICATION

(11) **EP 3 369 859 B1**
(45) Date of publication and mention of the grant of the patent: **20.09.2023**
(21) Application number: 15906939.2
(22) Date of filing: 28.10.2015
(51) Int. Cl.: D06M 13/188, D06M 11/13, D01C 3/00, D02J 1/22, D06M 13/00, D06M 10/04, D06M 11/55, D06M 11/70, D06M 13/21

(54) **HIGH PERFORMANCE NATURAL SILK FIBER AND PREPARATION METHOD THEREOF**
NATÜRLICHE HOCHLEISTUNGSSEIDENFASER UND HERSTELLUNGSVERFAHREN DAFÜR
FIBRE DE SOIE NATURELLE DE HAUTE PERFORMANCE ET SON PROCÉDÉ DE PRÉPARATION

(43) Date of publication of application: 05.09.2018
(73) Proprietor: Nantong Textile & Silk Industrial Technology Research Institute, Jiangsu 226300 (CN)
(72) Inventor: ZHANG, Feng, Nantong Jiangsu 226300 (CN); ZUO, Baoqi, Nantong Jiangsu 226300 (CN)
(74) Representative: Lang, Christian
(86) International application number: PCT/CN2015/093139
(87) International publication number: WO 2017/070873

(56) References cited:
- CN-A- 101 545 146
- CN-A- 101 545 146
- CN-A- 103 469 563
- CN-A- 105 256 544
- GB-A- 283 481
- GB-A- 485 398
- JP-B2- H0 141 754
- US-A- 2 072 155
- FENG ZHANG ET AL: "Facile Fabrication of Robust Silk Nanofibril Films via Direct Dissolution of Silk in CaCl 2 -Formic Acid Solution", ACS APPLIED MATERIALS & INTERFACES, vol. 7, no. 5, 29 January 2015 (2015-01-29), pages 3352-3361, XP055586959, US ISSN: 1944-8244, DOI: 10.1021/am508319h

## Description

### Technical field

The invention belongs to the field of natural polymer materials, and in particular relates to a high-performance natural silk fiber and a preparation method thereof.

### Background technique

Silk is a continuous long fiber made from the coagulation of silk glands secreted from jujube when silkworm is cooked and is one of the earliest animal fibers to be used in human beings. According to different foods, silk is divided into mulberry silk, tussah silk, silk and eri silk. The strands drawn from a single silkworm cocoon are called cocoon filaments, which consist of two monofilaments that are adhesively coated with sericin. The silkworms of several silkworm cocoons were withdrawn, and the silks wrapped by silk adhesive were called raw silk. Several raw silks are processed through the process of collateral, twisting, weaving, or weaving to become twisted or braided stitches. As a high-grade textile raw material, silk products are deeply loved by consumers at home and abroad.

In recent years, with the development of polymer science and cross-infiltration among disciplines, the application of silk materials is infiltrating from traditional textiles to high-tech fields. Among them, the research of high-performance silk fibers is one of the hot spots. As a non-physiological structural protein macromolecule, the mechanical properties of silk are closely related to the aggregation structure. Spider silk has particularly excellent mechanical properties, such as high strength, high modulus, high elongation, high fracture work, and has great application value and prospects in high-tech fields such as body armor and sutures. Therefore, it has become a hot topic for material scientists today. It was found that the fiber of the best mechanical property is spider silk, which is also a non-physiologically active structural protein polymer. However, the spiders are killing to each other and cannot be mass-produced in large quantities like silkworms. It has been considered that the reason why the mechanical properties of silk is far inferior to that of spider silk is that the primary structure of silk and spider silk (also known as amino acid composition and sequence distribution) is very different.

For this purpose, the researchers implanted genes of spider which produces spider silk into silkworm to produce silk containing spider silk protein. Compared with ordinary silk, the mechanical properties improved significantly, such as the strength increase of about 20%, the elongation rate increased by about 30%. The high-performance silk fiber has broad application prospects in body armor, high-strength ultra-fine sutures, artificial ligaments, and tendons. The purpose of the transgenic technology is to transform the primary structure of silk. Although progress has been made in this area, major breakthroughs have not yet been made and industrialization cannot be achieved. NATURE magazine published in 2002 published the papers of Professor Shao Zhengzhong from Fudan University and Professor Vollrath from Oxford University in the UK. They used the forced-pulling process to make the silkworm spit out the natural silk that is comparable to spider silk [Shao Z, et al. Nature 2002; 418: 741.]. This study shows that the difference in the mechanical properties of silk and spider silk is mainly caused by the structural differences of secondary structure of fibrin or above secondary structure of fibrin. This difference can be reduced or eliminated by changes in silkworm silking behavior, so as to obtain spider silk with excellent mechanical properties. However, because silkworm larvae are small and soft, have strong head movements, and silk is delicate and easily broken, it is not feasible to mass-produce spider silk by altering silkworm silking behavior.

The difference in the speed of silk threading mainly affects the molecular orientation structure and part of the crystal structure of the silk protein, resulting in a change in the mechanical properties of the silk. Natural silk fiber, thanks to its unique multi-level structure, has excellent mechanical properties in itself. The performance improvement based on this is the best way to prepare high-performance silk protein fibers. The results of strong spinning should be obtained as well theoretically by reorganization of the natural silk structure and further transformation of the silk by the stretching and setting process. However, the formed natural silk fibers are mainly anti-parallel β-sheet crystal structures, and their aggregation structure is very stable, which is difficult to change, perform physical stretching post-treatment cannot be used in the prior art. In the prior art, the natural silk is generally dissolved and then spun to obtain a product with higher performance; however, due to the irreversible destruction of the multi-stage structure of the silk by the dissolving solvent and the spinning solvent, such as a decrease in the molecular weight, disintegration of the fibril structure, etc., caused the fiber structure of regenerated silk is unstable and the mechanical properties are poor. Although the mechanical properties of the regenerated silk fiber can be improved by post-stretching, the performance improvement is limited, not to mention that it is a fiber with better mechanical properties than the natural silk fiber. Therefore, the search for a method for reconstructing natural silk structure to obtain high-performance natural silk fibers has important value and significance for the application of silk in high-tech fields.Document CN 101 545 146 A discloses a method for improving silk fiber strength, comprising the steps of, firstly, providing a silk swelling liquid containing a base. Secondly, a silk fiber to be treated is soaked in said silk swelling liquid, the soaking time being 30 minutes. This is followed by stretching the soaked silk fibers. Finally, the stretched silk fiber is naturally air-dried under the condition of maintaining tension, thereby obtaining silk fiber with high crystallinity and high strength. By using natural drying after stretching and maintaining tension under the condition of stretching and maintaining silk fibroin, crystallinity and orientation of silk fibers are improved. Thereby the strength of the silk fiber can be increased by 20 to 75 %, wherein swelling under the defined conditions is used to simulate the state of silk fibroin and sericin in the silkworm body, thereby increasing the stretching speed. Since the higher the stretching speed, the greater the strength increase, high-strength silk fibers may be obtained. The article "Facile Fabrication of Robust Silk Nanofibril Films via Direct Dissolution of Silk in CaCl 2 - Formic Acid Solution", Zeng et al., ACS APPLIED MATERIALS & INTERFACES, vol. 7, no. 5, 29 January 2015 (2015-01-29), pages 3352-3361, DOI: 10.1021/am508319h discloses a method for preparing novel silk fibroin (SF) nanofibrous films with robust mechanical properties, including the steps of firstly degumming silk and then, dissolving the degummed silk in a CaCl2 - formic acid solution. The degummed silk (not the natural silk fiber) is dissolved in the solution, wherein during the dissolution process, swelling occurs. Formic acid is then evaporated within 24 h. The resulting SF films are washed in water for 2 h to remove CaCl2 and excess acid and induce β-sheet structure. The films are then air-dried and vacuum-dried. Cast films can be additionally stretched to modify properties.

### Summary of the Invention

The object of the invention is to provide a high-performance natural silk fiber and a preparation method thereof. The fiber is obtained by direct treatment of natural silk and has excellent mechanical properties, and can be widely used in civilian and military protection fields.

The invention as defined in the claims achieves the purpose of the invention.

Preferably, the acid in step (1) is one or more of formic acid, trifluoroacetic acid, acetic acid, hydrofluoric acid, phosphoric acid, and sulfuric acid; the concentration of the acid is 10% to 99% by weight.

More preferably, the acid is one of formic acid, hydrofluoric acid, phosphoric acid, and sulfuric acid; the concentration of the acid is 25% to 98% by weight.

In a preferred technical solution, wherein in step (1), the silk swelling liquid further comprises an inorganic salt; the concentration of the inorganic salt is 0.1% to 10% by weight; the inorganic salt is one or more of sodium chloride, potassium chloride, lithium bromide, calcium chloride, zinc chloride, magnesium chloride, lithium thiocyanate, sodium thiocyanate, magnesium thiocyanate, calcium nitrate, copper nitrate, calcium carbonate, and calcium phosphate. Preferably, the silk swelling liquid further comprises an inorganic salt; the inorganic salt is one of the lithium bromide, calcium chloride, magnesium chloride, and lithium thiocyanate; the concentration of the inorganic salt is 0.5% to 5% by weight.

The silk in the invention is a natural silk, which is unregenerated treatment, and it is selected from one or more of mulberry silk, tussah silk, yamamai silk, and eri silk. The natural silk fiber is one or more of silk, raw silk, twisted silk, and braided silk.

In the technical solution above, wherein in the step (2), the shrinkage during the shrinkage is 1% to 80% and the draw-ratio during the stretching is 1.1 to 5. In invention, the natural silk fiber can be stretched or shrunk while being soaked, or it can be stretched or shrunk after the natural silk fiber is soaked.

Preferably, the shrinkage during the shrinkage is 20% to 70%; and the draw-ratio during the stretching is 1.1 to 3.2; the soaking time is 5 seconds to 5 minutes.

The invention performs physical stretching/shrinkage modification on natural silk fibers (including silk, raw silk, twisted silk, braided silk, etc.), breaks through the technical problem that natural silk fibers cannot be stretched, and achieves a huge leap of the mechanical properties of natural silk fibers, to meet the application requirements of silk in special areas such as body armor, artificial ligaments, and ophthalmic sutures. Therefore, the invention also discloses a high performance natural silk fiber prepared according to the above preparation method.

### The advantages of the invention

### Advantages

Owing to the application of the technical solution above, compared with the prior art, this invention has the advantages as follow:
(1)The invention realizes the direct drawing treatment of natural silk fibers for the firs t time, thereby achieving the effect of improving the mechanical properties of natural silk, the breaking strength reaching more than 1000 MPa and the breaking elongation reaching 50% or more; overcoming the technical problem that the existing natural silk cannot stretching and achieved unexpected technical effects.
(2) The invention overcomes the defect that the prior art mainly deals with the transgene or forced wire drawing of silkworms. Compared with the prior art, the breaking strength of the natural silk obtained by the invention can be increased by a factor of 2 and can reach 1 GPa or more, and can be used for making high-performance raw silk, twisted silk, braided silk, etc., in line with production applications.
(3) The method selected suitable solvent parameters and dissolving conditions to make silkworm insolubilization and removing β-folded structure, thus providing a window for the structure modification and performance adjustment of natural silk fibers, and obtaining high performance natural silk fibers by simple method.

The processing method to improve the strength of natural fiber is simple and efficient, and can be directly connected with the production line of the existing product to realize large-scale production of high performance natural silk fiber.

### Description of the drawings

FIG. 1 is a scanning electron microscopy image of a surface of a natural silk fiber before and after treatment in Example 1;
FIG. 2 is a scanning electron micrograph of the cross section of the natural silk fiber before and after the treatment in Example 1;
FIG. 3 is an infrared spectrum of a natural silk fiber before and after treatment in Example 2;
FIG. 4 is a Raman spectrum before and after treatment of natural silk fibers in Example 2.

### Detailed description

The invention will be further described below with reference to the accompanying drawings and embodiments.

### Example 1

(1) Confect the natural silk swelling liquid: formic acid of 98 wt% is diluted with water to 80%, and then add lithium bromide in to get 80% formic acid solution containing 2% lithium bromide, which is the silk swelling liquid;
(2) Immerse mulberry silk in swelling liquid of the step (1)for 30 seconds, and at the same time control the silk to shrink to 60% of the original length, to obtain shrink silk;
(3) After washed with deionized water, shrink silk by the step (2) is neutralized the excess acid in aqueous sodium hydroxide solution with 1wt%, and then washed again and dried in the oven at 60°C, get high performance natural silk fiber.

Table 1 shows the mechanical tensile data of mulberry silk before and after treatment. According to the technical scheme provided by the present invention, the cocoon silk after treatment has excellent ductility, and the elongation at break reaches more than 50%.

**Table 1 Mechanical tensile data of mulberry silk before and after processing**

| Sample | Elongation at Break (%) | Fracture work (MJ/m³) |
|---|---|---|
| Original mulberry silk | 21.1 | 64.5 |
| Handle mulberry silk | 52.3 | 72.8 |

FIG. 1, FIG. 2 and Table 1 are scanning electron microscope and mechanical tensile properties data of the above-mentioned high performance natural silk fiber before and after treatment. As can be seen from Fig. 1, the arrow of the solid line is the fiber direction. After processing, the highly ordered nanofibril orientation structure inside the silk is destroyed; as can be seen from Fig. 2, the nanofibrillar structure inside the silkworm cocoon becomes fluffy and clearly visible; the invention effectively removes the natural silk β-sheet structure, thereby greatly improving the performance of the natural silk fiber. In addition, as can be seen from Table 1, after treatment, the elongation of natural mulberry silk is significantly increased to more than 50%, and the work of fracture is improved by about 10%.

### Example 2

(1) Confect the natural silk swelling liquid: formic acid of 98 wt% is diluted with water to 80%, and then adds calcium chloride in to get 80% formic acid solution containing 2% calcium chloride, which is the silk swelling liquid;
(2) Immerse mulberry silk in swelling liquid of the step (1) for 30 seconds, and then stretch the silk to twice the original length, to obtain stretching silk;
(3) After washed with deionized water, stretching silk by the step (2) is neutralized the excess acid in the 1wt% aqueous sodium hydroxide solution, and then washed again and dried in the oven at 60°C, get high performance natural silk fiber.

Table 2 shows the mechanical tensile data of the mulberry silk before and after the treatment. According to the technical scheme provided by the present invention, the silk has excellent strength and the breaking strength reaches 900 MPa or more.

**Table 2 Mechanical tensile data before and after processing**

| Sample | Breaking strength (MPa) |
|---|---|
| Original mulberry silk | 450 |
| Stretching mulberry silk | 920 |

FIG. 3, FIG. 4 and Table 2 are the infrared spectra, Raman spectra and mechanical properties of the above-mentioned high-performance natural silk fiber before and after the treatment. As can be seen from Fig. 3, after treatment, the crystallinity inside the silk was destroyed, which was significantly reduced compared with that before treatment. From Fig. 4, it can be seen that the molecular orientation degree of the silk fiber is significantly increased after stretched; this is favorable for the improvement of mechanical properties of natural silk. In addition, as can be seen from Table 2, after the stretching treatment, the breaking strength of the silk was significantly improved, and the breaking strength was 800 MPa or more.

### Example 3

(1) Confect the natural silk swelling liquid: add lithium thiocyanate into formic acid of 98 wt% to get formic acid solution which containing 1% lithium thiocyanate, that is the silk swelling liquid;
(2) Immerse 20-22D raw silk in swelling liquid of the step (1)for 50 seconds, and then control the raw silk to shrink to 30% of the original length, to obtain shrink raw silk;
(3) After washed with deionized water shrink, raw silk by the step (2) is neutralized the excess acid in the 1wt% aqueous sodium hydroxide solution, and then washed again and dried in the oven at 70°C, get high performance natural silk fiber.

Table 3 shows the mechanical tensile data of the raw silk before and after the treatment. According to the technical scheme provided by the present invention, the raw silk processed has excellent ductility, the elongation at break reaches above 50%, and the work of fracture increases by about 20%.

**Table 3 Mechanical tensile data of raw silk before and after treatment**

| Sample | Elongation at Break (%) | Fracture work (MJ/m³) |
|---|---|---|
| Original raw silk | 21.1 | 354.2 |
| Handle raw silk | 58.5 | 412.8 |

### Example 4

(1) Confect the natural silk swelling liquid: add magnesium chloride into trifluoroacetic acid of 90 wt% to get hydrofluoric acid solution which containing 1% magnesium chloride, that is the silk swelling liquid;
(2) Immerse 20-22D raw silk in swelling liquid of the step (1) for 50 seconds, and while stretch the raw silk to 1.5 times the original length, to obtain stretching raw silk;
(3) After washed with deionized water stretching silk by the step (2), is neutralized the excess acid in aqueous sodium hydroxide solution of 1wt%, and then washed again and dried in the oven at 55°C, get high performance natural silk fiber.

Table 4 shows the mechanical tensile data of the raw silk before and after the treatment. According to the technical scheme provided by the present invention, the raw silk processed has excellent strength, and the breaking strength is more than 800 MPa.

**Table 4 Mechanical tensile data of raw silk before and after treatment**

| Sample | Breaking strength (cN) |
|---|---|
| Raw silk | 81.2 |
| Stretching silk | 105.6 |

### Example 5

(1) Confect the natural silk swelling liquid: dilute formic acid of 98 wt% to 90 wt%, which is the silk swelling liquid;
(2) Immerse the braided silk with the diameter is about 0.22mm in swelling liquid of the step (1) for 20 seconds, and while stretch the raw silk to 1.3 times the original length, to obtain stretching braided silk;
(3) After washed with deionized water stretching braided silk by the step (2), is neutralized the excess acid in the 1wt% aqueous sodium hydroxide solution, and then washed again and dried in the oven at 60°C, get high performance natural silk fiber.
Table 5 shows the mechanical tensile data of the braided silk before and after the treatment. According to the technical solution provided by the present invention, the breaking strength of the stretched braided sutures is significantly increased and reaches over 3000 cN.

**Table 5 Mechanical tensile data before and after treatment of braided silk**

| Sample | Breaking strength (cN) |
|---|---|
| Original braided silk (4#) | 2787.8 |
| Stretching braided silk | 3875.6 |

### Example 6

(1) Confect the natural silk swelling liquid: dilute concentrated sulfuric acid to 30wt%, which is the silk swelling liquid;
(2) Immerse tussah silk in swelling liquid of the step (1) for 50 seconds, and then stretch to 3 times the original length, to obtain stretching silk;
(3) After washed with deionized water stretching silk by the step (2), is neutralized the excess acid in the 1wt% aqueous sodium hydroxide solution, and then washed again and dried in the oven at 60°C, get high performance natural silk fiber.

Table 6 shows the mechanical tensile data of the tussah silk before and after the treatment. According to the technical scheme provided by the present invention, the tensile strength of the stretched tussah silk is significantly improved and reaches above 1000 MPa.

**Table 6 Mechanical tensile data of tussah silk before and after treatment**

| Sample | Breaking strength (MPa) |
|---|---|
| Original tussah silk | 430 |
| Stretching tussah silk | 1100 |

### Example 7

(1) Confect the natural silk swelling liquid: dilute concentrated phosphoric acid to 25wt%, which is the silk swelling liquid;
(2) Immerse eri silk in swelling liquid of the step (1) for 30 seconds, and then stretch to 2 times the original length, to obtain stretching eri silk;
(3) After washed with deionized water stretching eri silk by the step (2), is neutralized the excess acid in 1wt% aqueous sodium hydroxide solution, and then washed again and dried in the oven at 60°C, get high performance natural silk fiber.

Table 7 shows the mechanical tensile data of the eri silk before and after the treatment. According to the technical scheme provided by the present invention, the breaking tussah silk filament rupture strength is significantly improved and reaches 780 MPa or more.

**Table 7 Mechanical tensile data of eri silk before and after treatment**

| Sample | Breaking strength (MPa) |
|---|---|
| Original eri silk | 463 |
| Stretching eri silk | 783 |

The concentrations in this example are all mass concentrations. The present invention can modify the mechanical properties of existing natural silk fiber products (including silk, raw silk, twisted silk, and braided silk etc.) to construct a natural silk fiber with high performance and high elongation.

## Claims

1. A method for preparing high-performance natural silk fiber, comprising the following steps:
(1) Preparing a silk swelling liquid, the silk swelling liquid comprising acid and water;
(2) Soaking a natural silk fiber in the silk swelling liquid of step (1), the soaking time being 5 seconds to 5 minutes, and shrinking or stretching the soaked natural silk fibers;
(3) Washing the treated natural silk fiber obtained in step (2) with deionized water, neutralizing the excess acid in an aqueous sodium hydroxide solution of 1 wt.-%, washing again with water, and drying in an oven at a specific temperature of 55 °C, 60 °C or 70 °C to obtain the high performance natural silk fiber, in which the natural silk β-sheet structure is removed.

2. The method for preparing high-performance natural silk fiber according to claim 1, wherein in step (1), the acid is one or more of formic acid, trifluoroacetic acid, acetic acid, hydrofluoric acid, phosphoric acid, and sulfuric acid; the concentration of the acid being 10% to 99% by weight.

3. The method for preparing high-performance natural silk fiber according to claim 2, wherein in step (1), the acid is one of formic acid, hydrofluoric acid, phosphoric acid, and sulfuric acid; the concentration of the acid being 25% to 98% by weight.

4. The method for preparing high-performance natural silk fiber according to claim 1, wherein in step (1), the silk swelling liquid further comprises an inorganic salt; the inorganic salt being one or more selected from sodium chloride, potassium chloride, lithium bromide, calcium chloride, zinc chloride, magnesium chloride, lithium thiocyanate, sodium thiocyanate, magnesium thiocyanate, calcium nitrate, copper nitrate, calcium carbonate and calcium phosphate; the concentration of the inorganic salt being 0.1% to 10% by weight.

5. The method for preparing high-performance natural silk fiber according to claim 4, wherein in step (1), the silk swelling liquid further comprises an inorganic salt; the inorganic salt being one of lithium bromide, calcium chloride, magnesium chloride and lithium thiocyanate; the concentration of the inorganic salt being 0.5% to 5% by weight.

6. The method for preparing high-performance natural silk fiber according to claim 1, wherein in step (2), the natural silk is one or more of mulberry silk, tussah silk, yamamai silk, and eri silk.

7. The method for preparing high-performance natural silk fiber according to claim 1, wherein in step (2), the natural silk fiber is one or more of silk, raw silk, twisted silk, and braided silk.

8. The method for preparing high-performance natural silk fiber according to claim 1, wherein in the step (2), the shrinkage during the shrinkage is 1% to 80%; and the draw-ratio during the stretching is 1.1 to 5.

9. The method for preparing high-performance natural silk fiber according to claim 8, wherein in step (2), the shrinkage during the shrinkage is 20% to 70%; and the draw-ratio during the stretching is 1.1 to 3.2.

10. The high-performance natural silk fiber prepared by the preparation method according to any one of claim 1 to 9, **characterized in that** in the high-performance natural silk fiber the natural silk β-sheet structure is removed.

## Patentansprüche

1. Ein Verfahren zur Herstellung einer Hochleistungs-Naturseidenfaser, umfassend die folgenden Schritte:
(1) Herstellen einer Seidenquellflüssigkeit, wobei die Seidenquellflüssigkeit Säure und Wasser enthält;
(2) Einweichen einer Naturseidenfaser in der Seidenquellflüssigkeit von Schritt (1), wobei die Einweichzeit 5 Sekunden bis 5 Minuten beträgt, und Schrumpfen oder Strecken der eingeweichten Naturseidenfasern;
(3) Waschen der in Schritt (2) erhaltenen behandelten Naturseidenfaser mit entionisiertem Wasser, Neutralisieren der überschüssigen Säure in einer wässrigen Natriumhydroxidlösung von 1 Gew.-%, erneutes Waschen mit Wasser und Trocknen in einem Ofen bei einer spezifischen Temperatur von 55°C, 60°C oder 70°C, um die Hochleistungs-Naturseidenfaser zu erhalten, bei der die Naturseiden-β-Schichtstruktur entfernt ist.

2. Das Verfahren zur Herstellung einer Hochleistungs-Naturseidenfaser nach Anspruch 1, wobei in Schritt (1) die Säure eine oder mehrere von Ameisensäure, Trifluoressigsäure, Essigsäure, Fluorwasserstoffsäure, Phosphorsäure und Schwefelsäure ist, wobei die Konzentration der Säure 10 Gew.-% bis 99 Gew.- % beträgt.

3. Das Verfahren zur Herstellung einer Hochleistungs-Naturseidenfaser nach Anspruch 2, wobei in Schritt (1) die Säure eine von Ameisensäure, Fluorwasserstoffsäure, Phosphorsäure und Schwefelsäure ist, wobei die Konzentration der Säure 25 Gew.-% bis 98 Gew.-% beträgt.

4. Das Verfahren zur Herstellung einer Hochleistungs-Naturseidenfaser nach Anspruch 1, wobei in Schritt (1) die Seidenquellflüssigkeit weiterhin ein anorganisches Salz enthält; wobei das anorganische Salz eines oder mehrere ist, ausgewählt aus Natriumchlorid, Kaliumchlorid, Lithiumbromid, Calciumchlorid, Zinkchlorid, Magnesiumchlorid, Lithiumthiocyanat, Natriumthiocyanat, Magnesiumthiocyanat, Calciumnitrat, Kupfernitrat, Calciumcarbonat und Calciumphosphat; wobei die Konzentration des anorganischen Salzes 0,1 Gew.-% bis 10 Gew.-% beträgt.

5. Das Verfahren zur Herstellung einer Hochleistungs-Naturseidenfaser nach Anspruch 4, wobei in Schritt (1) die Seidenquellflüssigkeit weiterhin ein anorganisches Salz umfasst, wobei das anorganische Salz eines von Lithiumbromid, Calciumchlorid, Magnesiumchlorid und Lithiumthiocyanat ist, wobei die Konzentration des anorganischen Salzes 0,5 Gew.-% bis 5 Gew.-% beträgt.

6. Das Verfahren zur Herstellung einer Hochleistungs-Naturseidenfaser nach Anspruch 1, wobei in Schritt (2) die Naturseide eine oder mehrere von Maulbeerseide, Tussah-Seide, Yamamai-Seide und Eri-Seide ist.

7. Das Verfahren zur Herstellung einer Hochleistungs-Naturseidenfaser nach Anspruch 1, wobei in Schritt (2) die Naturseidenfaser eine oder mehrere von Seide, Rohseide, gedrehter Seide und geflochtener Seide ist.

8. Das Verfahren zur Herstellung einer Hochleistungs-Naturseidenfaser nach Anspruch 1, wobei in Schritt (2) die Schrumpfung während des Schrumpfens 1% bis 80% beträgt; und das Streckverhältnis während des Streckens 1,1 bis 5 beträgt.

9. Das Verfahren zur Herstellung einer Hochleistungs-Naturseidenfaser nach Anspruch 8, wobei in Schritt (2) die Schrumpfung während des Schrumpfens 20% bis 70% beträgt und das Streckverhältnis während des Streckens 1,1 bis 3,2 beträgt.

10. Das Hochleistungs-Naturseidenfaser, hergestellt nach dem Herstellungsverfahren gemäß einem der Ansprüche 1 bis 9, **dadurch gekennzeichnet, dass** in der Hochleistungs-Naturseidenfaser die Naturseiden-β-Schichtstruktur entfernt ist.

## Revendications

1. Procédé de préparation d'une fibre de soie naturelle de haute performance, comprenant les étapes suivantes consistant à :
(1) préparer un liquide de gonflement de soie, le liquide de gonflement de soie comprenant de l'acide et de l'eau ;
(2) tremper une fibre de soie naturelle dans le liquide de gonflement de soie de l'étape (1), le temps de trempage étant compris entre 5 secondes et 5 minutes, et rétrécir ou étirer les fibres de soie naturelle trempées ;
(3) laver la fibre de soie naturelle traitée obtenue à l'étape (2) avec de l'eau désionisée, neutraliser l'excès d'acide dans une solution aqueuse d'hydroxyde de sodium de 1 % en poids, laver à nouveau avec de l'eau et sécher dans un four à une température spécifique de 55 °C, 60 °C ou 70 °C pour obtenir la fibre de soie naturelle de haute performance, dans laquelle la structure à feuillets β de la soie naturelle est éliminée.

2. Procédé de préparation d'une fibre de soie naturelle de haute performance selon la revendication 1, dans lequel, à l'étape (1), l'acide est un ou plusieurs parmi l'acide formique, l'acide trifluoroacétique, l'acide acétique, l'acide fluorhydrique, l'acide phosphorique et l'acide sulfurique ; la concentration de l'acide étant de 10 % à 99 % en poids.

3. Procédé de préparation d'une fibre de soie naturelle de haute performance selon la revendication 2, dans lequel, à l'étape (1), l'acide est l'un parmi l'acide formique, l'acide fluorhydrique, l'acide phosphorique et l'acide sulfurique ; la concentration de l'acide étant de 25 % à 98 % en poids.

4. Procédé de préparation d'une fibre de soie naturelle de haute performance selon la revendication 1, dans lequel, à l'étape (1), le liquide de gonflement de soie comprend en outre un sel inorganique ; le sel inorganique étant un ou plusieurs sélectionnés parmi le chlorure de sodium, le chlorure de potassium, le bromure de lithium, le chlorure de calcium, le chlorure de zinc, le chlorure de magnésium, le thiocyanate de lithium, le thiocyanate de sodium, le thiocyanate de magnésium, le nitrate de calcium, le nitrate de cuivre, le carbonate de calcium et le phosphate de calcium ; la concentration du sel inorganique étant de 0,1 % à 10 % en poids.

5. Procédé de préparation d'une fibre de soie naturelle de haute performance selon la revendication 4, dans lequel, à l'étape (1), le liquide de gonflement de soie comprend en outre un sel inorganique ; le sel inorganique étant l'un parmi le bromure de lithium, le chlorure de calcium, le chlorure de magnésium et le thiocyanate de lithium ; la concentration du sel inorganique étant de 0,5 % à 5 % en poids.

6. Procédé de préparation d'une fibre de soie naturelle de haute performance selon la revendication 1, dans lequel, à l'étape (2), la soie naturelle est une ou plusieurs parmi la soie de mûrier, la soie tussah, la soie yamamai et la soie eri.

7. Procédé de préparation d'une fibre de soie naturelle de haute performance selon la revendication 1, dans lequel, à l'étape (2), la fibre de soie naturelle est une ou plusieurs parmi la soie, la soie brute, la soie torsadée et la soie tressée.

8. Procédé de préparation d'une fibre de soie naturelle de haute performance selon la revendication 1, dans lequel, à l'étape (2), le rétrécissement pendant le rétrécissement est de 1 % à 80 % ; et le rapport d'étirage pendant l'étirement est de 1,1 à 5.

9. Procédé de préparation d'une fibre de soie naturelle de haute performance selon la revendication 8, dans lequel, à l'étape (2), le rétrécissement pendant le rétrécissement est de 20 % à 70 % ; et le rapport d'étirage pendant l'étirement est de 1,1 à 3,2.

10. Fibre de soie naturelle de haute performance préparée par le procédé de préparation selon l'une quelconque des revendications 1 à 9, **caractérisée en ce que**, dans la fibre de soie naturelle de haute performance, la structure à feuillets β de la soie naturelle est éliminée.
